

Sept. 28, 1948.

H. L. GIBBS

2,449,984

DIFFERENTIAL FROTH FLOTATION OF SULFIDE ORES

Filed April 10, 1944



Inventor:

H. L. GIBBS,

By *H. L. Gibbs*  
*B. Mallinckrodt and*  
*Philip A. Mallinckrodt*

Attorney

## UNITED STATES PATENT OFFICE

2,449,984

DIFFERENTIAL FROTH FLOTATION OF  
SULFIDE ORES

Harold L. Gibbs, Salt Lake City, Utah

Application April 10, 1944, Serial No. 530,389

23 Claims. (Cl. 209—167)

1

This invention relates to a process of flotation for separating metalliferous sulphides one from another and from other minerals by which they may be accompanied, especially in the case of ore minerals and concentrates. Quite particularly, the process relates to froth flotation, and to the concentration of metalliferous sulphides such as those of molybdenum, copper, iron, zinc and lead.

More specifically the invention relates to the use of certain agents novel in flotation practice, by means of which some of the mineral values are depressed, while other minerals or impurities are caused to float by any usual flotation agents. The novel depressing agents are organic compounds each comprising two active groups, one a water wetting group and the other a mineral collector group, the two groups being chemically joined by an organic group or radical which is preferably otherwise inactive in the compound.

Primarily, among the important objects of the invention are the following:

An improvement in the separation of molybdenite from other sulphides principally copper and iron.

An improvement in agents by means of which the separation of certain metalliferous sulphides from other minerals is greatly facilitated.

An improvement that makes it possible to control the separation of molybdenite from other sulphides.

Other objects will appear when the process is fully understood.

In processes of flotation it is usual to float more than one mineral in the initial or rougher stage. In the flotation process of the invention, it is a distinctive feature to obtain a separation of these minerals by preventing the flotation of a particular mineral either in the initial flotation step or in a subsequent step.

The flotation of minerals in an aqueous pulp fundamentally depends upon the extent of water wetting or non-wetting of the mineral particles which it is desired to separate from other mineral particles. Thus in separating molybdenite from copper or iron sulphides, the purpose is to encourage the floating of the molybdenite by non-wetting the surfaces of the particles and to depress or inhibit the floating of the copper and iron sulphides by wetting the surfaces of those particles. It is to this latter purpose that the use of the novel agents of this invention are directed. By using well known agents to increase the floatability of a particular metalliferous sulphide and using the novel agents of the invention to depress certain other metalliferous sulphides, the process of the invention can be so adjusted that various metalliferous sulphides are profitably separated one from another.

I have discovered a particular group of organic compounds each of the members of which acts

very energetically to depress or prevent the flotation of copper sulphides and other sulphide minerals while at the same time allowing the flotation of molybdenite. This group of organic agents has the type formula  $HSRCOOH$  or a very similar type formula  $HSRCOSH$ , in both of which  $R$  represents an organic group, advantageously and for example, a saturated aliphatic group otherwise known as a saturated straight chain.

Various examples of chemical compounds under the type formula may be given as follows:

- (1)  $HS$   $R$   $COOH$  Type formula
- (2)  $HS$   $CH_2$   $COOH$  Thioglycolic acid
- (3)  $HS$   $CH$   $COOH$  Alpha mercapto butyric acid
- (4)  $HS$   $CH_2$   $COOH$  Alpha mercapto caproic acid
- (5)  $KS$   $C$   $COSK$  Potassium dithio oxalate

The type formula  $HSRCOOH$  is intended to include also the water soluble salts of these acids which may be formed either during their preparation or after being placed in the flotation pulp, because of the positive ions in the pulp. A particular example of this formation is in the agent potassium dithio oxalate,  $KSOCCOSK$ , where the potassium ion has replaced the hydrogen ion, also in mercapto caproic acid which was converted to the sodium salt before being used.

In applying the invention the depressing properties of thioglycolic acid on copper sulphide minerals have been investigated over a wide range of pH values including both acid and alkaline values. The value of pH is not a limiting factor at pH values lower than 9. Above a 9 pH the results become progressively poorer. As there is such a wide range of pH values at which this compound is effective as a depressant, the type of ore and previous treatment, as well as the particular depressant used, plays a part in establishing the optimum pH value.

The depression of copper sulphide minerals by thioglycolic acid is illustrated in the various examples which will follow presently.

A flotation concentrate to which the process of the invention has been applied with favorable results, is one produced by the Utah Copper Company. This particular concentrate consists mostly of copper sulphide minerals accompanied by a small percentage of molybdenite. As a rule the Utah Copper Company concentrate assays approximately 33 per cent copper and one per cent molybdenite, the flotation being accomplished by means of the usual agents, burner oil and an alcohol frother.

In two examples of using the process of the invention on Utah Copper Company concentrates, the tendency of the copper sulphide minerals to float with the molybdenite was successfully over-

come by the depressive action of thioglycollic acid while the molybdenite was unaffected and was floated with the usual collector agents. The two examples are recorded as follows:

from 1.49 per cent to 75.00 per cent. The progressive elimination of copper due to the depressing action of thioglycollic acid is clearly shown.

*Example No. 1*

|                                      | Per Cent Weight | Assay, Per Cent |        |                  | Per Cent Distribution |        |                  |
|--------------------------------------|-----------------|-----------------|--------|------------------|-----------------------|--------|------------------|
|                                      |                 | Cu              | Insol. | MoS <sub>2</sub> | Cu                    | Insol. | MoS <sub>2</sub> |
| Heading (flotation concentrate)..... | 100.00          | 28.350          | 7.60   | 1.16             | 100.00                | 100.00 | 100.00           |
| Copper concentrate not floated.....  | 94.41           | 28.700          | 6.80   | 0.06             | 96.96                 | 89.55  | 4.94             |
| Molybdenite concentrate floated..... | 5.59            | 15.200          | 13.40  | 19.50            | 3.04                  | 10.45  | 95.06            |

In this example 96.96 per cent of the copper was depressed, while 95.06 of the molybdenite was floated. Flotation agents used were: 3.0 lbs.

Examples of the use of the other novel agents which satisfy the type formula, follow:

*Example No. 3*

|                                      | Per Cent Weight | Per Cent Assays |        |                  | Per Cent Distribution |        |                  |
|--------------------------------------|-----------------|-----------------|--------|------------------|-----------------------|--------|------------------|
|                                      |                 | Cu              | Insol. | MoS <sub>2</sub> | Cu                    | Insol. | MoS <sub>2</sub> |
| Heading (flotation concentrate)..... | 100.00          | 32.240          | 5.93   | 1.40             | 100.00                | 100.00 | 100.00           |
| Rougher tailing.....                 | 84.43           | 32.500          | 5.40   | 0.08             | 85.10                 | 76.88  | 4.83             |
| Cleaner tailing.....                 | 11.67           | 34.800          | 6.40   | 3.24             | 12.60                 | 12.60  | 27.06            |
| Molybdenite concentrate.....         | 3.90            | 19.000          | 16.00  | 24.40            | 2.30                  | 10.52  | 68.11            |

thioglycollic acid, 0.6 lb. burner oil, 0.2 lb. B-22 frother per ton.

Flotation agents in pounds per ton were added as follows:

*Example No. 2*

|                                      | Per Cent Weight | Per Cent Assays |        |                  | Per Cent Distribution |        |                  |
|--------------------------------------|-----------------|-----------------|--------|------------------|-----------------------|--------|------------------|
|                                      |                 | Cu              | Insol. | MoS <sub>2</sub> | Cu                    | Insol. | MoS <sub>2</sub> |
| Heading (flotation concentrate)..... | 100.00          | 32.850          | 7.40   | 1.49             | 100.00                | 100.00 | 100.00           |
| Rougher tailing.....                 | 93.55           | 33.535          | 7.20   | 0.16             | 94.59                 | 89.33  | 9.65             |
| 1st cleaner tailing.....             | 3.78            | 41.200          | 5.60   | 1.31             | 4.70                  | 2.81   | 3.19             |
| 2nd cleaner tailing.....             | 1.15            | 17.500          | 24.80  | 28.00            | 0.59                  | 3.78   | 20.76            |
| 3rd cleaner tailing.....             | 0.42            | 4.650           | 33.20  | 48.80            | 0.06                  | 1.84   | 13.21            |
| Molybdenite Conc.....                | 1.10            | 1.840           | 15.40  | 75.00            | 0.06                  | 2.24   | 53.19            |

In this example flotation agents in pounds per tons were added as follows:

|                  | Conc. H <sub>2</sub> SO <sub>4</sub> | Lime | Thioglycollic acid | Burner Oil | B-22  | Resulting pH | 55                   | Alpha Mercapto Butyric Acid | B-22 | Burner Oil | pH    |
|------------------|--------------------------------------|------|--------------------|------------|-------|--------------|----------------------|-----------------------------|------|------------|-------|
|                  |                                      |      |                    |            |       |              |                      |                             |      |            |       |
| Rougher.....     | 0.4                                  | 0.3  | 2.5                | 1.25       | 0.3   | 7.9          | Rougher tailing..... | 3.0                         | 0.27 | 0.5        | 7.8   |
| 1st cleaner..... | 0.2                                  | 0.15 | 0.35               | 0.08       | 0.045 | 8.0          | Cleaner tailing..... | 0.3                         | 0.09 | 0.5        | ----- |
| 2nd cleaner..... | 0.1                                  | 0.05 | 0.35               | 0.04       | 0.045 | 7.7          |                      |                             |      |            |       |
| 3rd cleaner..... | 0.1                                  | 0.05 | 0.35               | 0.08       | 0.045 | 7.5          |                      |                             |      |            |       |

Also in this example, several cleaning operations were made raising the per cent molybdenite

In this example it is shown that alpha mercapto butyric acid depresses 85.10 per cent of the copper per sulphides, while at the same time only 4.83 per cent of the molybdenite is prevented from floating.

*Example No. 4*

|                                      | Per Cent Weight | Per Cent Assays |        |                  | Per Cent Distribution |        |                  |
|--------------------------------------|-----------------|-----------------|--------|------------------|-----------------------|--------|------------------|
|                                      |                 | Cu              | Insol. | MoS <sub>2</sub> | Cu                    | Insol. | MoS <sub>2</sub> |
| Heading (flotation concentrate)..... | 100.00          | 44.950          | 4.40   | 1.50             | 100.00                | 100.00 | 100.00           |
| Rougher tailing.....                 | 16.42           | 35.900          | 14.00  | 0.86             | 13.33                 | 55.00  | 9.40             |
| Cleaner tailing.....                 | 54.36           | 47.300          | 2.60   | 0.86             | 58.15                 | 33.80  | 31.11            |
| Molybdenite concentrate.....         | 29.22           | 43.150          | 1.60   | 3.08             | 28.52                 | 11.20  | 59.49            |

Flotation agents in pounds per ton were added as follows:

|                 | Alpha Mercapto Caproic Acid <sup>1</sup> | B-22 | Burner Oil | pH   |
|-----------------|------------------------------------------|------|------------|------|
| Rougher tailing | 1.1                                      | 0.68 | 0.9        | 8.45 |
| Cleaner tailing | 1.1                                      | 0.34 | 0.9        | 8.3  |

<sup>1</sup> Neutralized with sodium hydroxide solution.

In this example it was found that the alpha mercapto caproic acid was largely insoluble in the flotation pulp, so that it was necessary to convert it into the sodium salt by reacting the acid with sodium hydroxide. The pronounced frothing properties of this compound limited the quantity that could be used, but in spite of the limitations the test shows the characteristic depressive action of substances coming under the type formula.

*Example No. 5*

|                                 | Per Cent Weight | Per Cent Assays |        |                  | Per Cent Distribution |        |                  |
|---------------------------------|-----------------|-----------------|--------|------------------|-----------------------|--------|------------------|
|                                 |                 | Cu              | Insol. | MoS <sup>2</sup> | Cu                    | Insol. | MoS <sup>2</sup> |
| Heading (flotation concentrate) | 100.00          | 44.950          | 4.40   | 1.50             | 100.00                | 100.00 | 100.00           |
| Rougher tailing                 | 91.50           | 42.250          | 4.00   | 0.14             | 94.53                 | 82.36  | 7.48             |
| Cleaner tailing                 | 5.32            | 34.900          | 8.40   | 8.20             | 4.24                  | 10.06  | 25.48            |
| Molybdenite concentrate         | 3.18            | 16.950          | 10.60  | 33.10            | 1.23                  | 7.58   | 67.04            |

Flotation agents in pounds per ton were added as follows:

|         | Potassium Dithio Oxalate | B-22 | Burner Oil | pH   |
|---------|--------------------------|------|------------|------|
| Rougher | 3.37                     | 0.34 | 0.6        | 8.45 |
| Cleaner | 2.25                     | 0.34 | 0.3        | 8.45 |

This example shows potassium dithio oxalate to have an effective depressive action upon copper sulphide minerals and gives further proof as to the reliability of the type formula.

These examples indicate that the novel depressants of the invention are effective with lead and zinc sulphides. The lead and zinc concentrates used in these tests were obtained by a well known method of flotation. In each case the novel depressants were added separately to the concentrate to depress the lead and zinc. Example 6 shows the percentage of lead and zinc floated by the well known method of flotation and Example 7 the percentage of lead and zinc depressed by my novel depressants.

*Example No. 6*

|              | Percent |
|--------------|---------|
| Lead floated | 98.34   |
| Zinc floated | 96.99   |

*Example No. 7*

|                | Percent |
|----------------|---------|
| Lead depressed | 95.21   |
| Zinc depressed | 94.35   |

Another example, numbered "8" which follows, represents two tests made relative to an ore containing a considerable amount of pyrite. Both the tests included in Example 8 were made under similar conditions, the difference in the two being that in the first test no thioglycollic acid was used, while in the second test thioglycollic acid was added after the pulp was agitated in the presence of ethyl xanthate. Flotation agents common to both tests include 3.25 lbs. lime, 0.1 lb. ethyl xanthate, 0.33 lb. frother (50 per cent

cresylic acid, 25 per cent amyl alcohol No. 44, 25 per cent B-22 frother) per ton of ore.

In the first test, i. e. where thioglycollic acid was not added the xanthate floated 30.85 per cent of the iron, while in the second test, i. e. where thioglycollic acid was added, only 5.54 per cent of the iron floated.

*Example No. 8*

| 10                                      | Per Cent Weight            | Per Cent Assays |       | Per Cent Distribution |
|-----------------------------------------|----------------------------|-----------------|-------|-----------------------|
|                                         |                            | Cu              | Fe    |                       |
| 15                                      | Without Thioglycollic acid |                 |       |                       |
| Heading                                 | 100.00                     | 0.500           | 2.35  | 100.00                |
| Rougher Tailings                        | 94.77                      | -----           | 1.70  | 69.15                 |
| Rougher Concentrate                     | 5.23                       | -----           | 13.75 | 30.85                 |
| With 0.6 lb. Thioglycollic Acid per ton |                            |                 |       |                       |
| Rougher Tailings                        | 97.33                      | -----           | 2.20  | 94.46                 |
| Rougher Concentrate                     | 2.67                       | -----           | 4.70  | 5.54                  |

In the accompanying drawing, which illustrates an instance of applying the process of the invention to actual practice, the single figure is a flow diagram representing a flotation plant using the novel process of the invention.

Referring to the drawing, the numeral 10 indicates a feed of aqueous flotation pulp consisting of molybdenite and copper sulphide minerals, the feed containing approximately 33 per cent Cu and one per cent MoS<sub>2</sub>. The feed enters the flotation circuit at 26, is acid conditioned at 27, and lime conditioned at 28. Farther on, for example at 29, a novel depressant agent is added after which the pulp at 30 enters the flotation section 31, the molybdenite concentrate (float) being discharged at 32 while the copper concentrate (sink) is discharged at 34.

Briefly summarizing comparatively, the prior and new practices in treating Utah Copper Company flotation concentrate to separate the molybdenite from the copper sulphide minerals, it may be stated that the prior practice comprises two general steps. The first step involves the use of dextrine to prevent the flotation of the molybdenite while a portion of the copper minerals are removed as a froth. The second step involves the further raising in grade of the flotation tailing or low grade molybdenite concentrate by heating sufficiently to alter the surfaces of the copper minerals and render them unfloatable, after which the molybdenite is floated away from the copper minerals. As opposed to that procedure, the new practice according to the invention, comprises first conditioning the original flotation concentrate with acid and then with lime, followed by the addition to the flotation pulp of a novel flotation agent which causes the copper minerals to be depressed, whereupon the molybdenite is floated away from the copper minerals. Thus the new procedure eliminates one flotation step and the necessity of providing the heat-treating equipment.

The disclosure herein, though embodying

specific examples, is limited only by the following claims.

What I claim is:

1. In a process of flotation for the separation of metalliferous sulphides, the step of agitating and aerating an aqueous pulp containing said metalliferous sulphides, in the presence of a frothing and a collecting agent for one of the sulphides and, further, in the presence of a depressant selected from the group of compounds having the formula  $HS-R-COOH$ , wherein R is an organic radical.

2. In a process of flotation for the separation of molybdenite from copper, iron, and similar sulphide minerals, the step of agitating and aerating an aqueous pulp containing the same, in the presence of a frothing and a collecting agent for the molybdenite and, further, in the presence of a depressant selected from the group of compounds having the formula



wherein R is an organic radical.

3. In a process of flotation for the separation of metalliferous sulphides, the steps of, first, subjecting an aqueous pulp containing the said metalliferous sulphides to inorganic acid conditioning, second, subjecting the acid conditioned pulp to lime conditioning sufficient to bring the pulp to an alkaline state, and, third, subjecting the so conditioned pulp to agitation and aeration in the presence of a frothing and a collecting agent for one of the sulphides and, further, in the presence of a depressant selected from the group of compounds having the formula



wherein R is an organic radical.

4. In a process of flotation for the separation of molybdenite from copper, iron, and similar sulphide minerals, the steps of, first, subjecting an aqueous pulp containing the said metalliferous sulphides to inorganic acid conditioning, second, subjecting the acid conditioned pulp to lime conditioning sufficient to bring the pulp to an alkaline state, and, third, subjecting the so conditioned pulp to agitation and aeration in the presence of a frothing and a collecting agent for the molybdenite and, further, in the presence of a depressant selected from the group of compounds having the formula  $HS-R-COOH$ , wherein R is an organic radical.

5. In a process of flotation for the separation of metalliferous sulphides, the step of agitating and aerating an aqueous pulp containing said metalliferous sulphides, in the presence of a frothing and collecting agent for one of the sulphides and, further, in the presence of a depressant having the general formula  $HS-R-X$ , in which R is an organic radical and X is selected from the group, carbonylic radical and thiocarbonylic radical.

6. In a process of flotation for the separation of metalliferous sulphides, the step of agitating and aerating an aqueous pulp containing said metalliferous sulphides, in the presence of a frothing and a collecting agent for one of the sulphides and, further, in the presence of a depressant selected from the group of compounds having the formula  $HS-R-COSH$ , wherein R is an organic radical.

7. In a process of flotation for the separation of metalliferous sulphides, the step of agitating and aerating an aqueous pulp containing said metalliferous sulphides, in the presence of a

frothing and a collecting agent for one of the sulphides and, further, in the presence of potassium dithio oxalate (KSOCCOSK).

8. In a process of flotation for the separation of molybdenite from copper, iron, and similar sulphide minerals, the step of agitating and aerating an aqueous pulp containing the same, in the presence of a frothing and a collecting agent for the molybdenite and, further, in the presence of a depressant selected from the group of compounds having the formula  $HS-R-COSH$ , wherein R is an organic radical.

9. In a process of flotation for the separation of molybdenite from copper, iron, and similar sulphide minerals, the step of agitating and aerating an aqueous pulp containing the same, in the presence of a frothing and a collecting agent for the molybdenite and, further, in the presence of potassium dithio oxalate (KSOCCOSK).

10. In a process of flotation for the separation of metalliferous sulphides, the steps of, first, subjecting an aqueous pulp containing the said metalliferous sulphides to inorganic acid conditioning, second, subjecting the acid conditioned pulp to lime conditioning sufficient to bring the pulp to an alkaline state, and, third, subjecting the so conditioned pulp to agitation and aeration in the presence of a frothing and a collecting agent for one of the sulphides and, further, in the presence of a depressant selected from the group of compounds having the formula  $HS-R-COSH$ , wherein R is an organic radical.

11. In a process of flotation for the separation of metalliferous sulphides, the steps of, first, subjecting an aqueous pulp containing the said metalliferous sulphides to inorganic acid conditioning, second, subjecting the acid conditioned pulp to lime conditioning sufficient to bring the pulp to an alkaline state, and, third, subjecting the so conditioned pulp to agitation and aeration in the presence of a frothing and a collecting agent for one of the sulphides and, further, in the presence of a depressant selected from the group of compounds having the formula  $HS-R-COSH$ , wherein R is an organic radical.

12. In a process of flotation for the separation of molybdenite from copper, iron, and similar sulphide minerals, the steps of, first, subjecting an aqueous pulp containing the said metalliferous sulphides to inorganic acid conditioning, second, subjecting the acid conditioned pulp to lime conditioning sufficient to bring the pulp to an alkaline state, and, third, subjecting the so conditioned pulp to agitation and aeration in the presence of a frothing and a collecting agent for the molybdenite and, further, in the presence of a depressant selected from the group of compounds having the formula  $HS-R-COSH$ , wherein R is an organic radical.

13. In a process of flotation for the separation of molybdenite from copper, iron, and similar sulphide minerals, the steps of, first, subjecting an aqueous pulp containing the said metalliferous sulphides to inorganic acid conditioning, second, subjecting the acid conditioned pulp to lime conditioning sufficient to bring the pulp to an alkaline state, and, third, subjecting the so conditioned pulp to agitation and aeration in the presence of a frothing and a collecting agent for the molybdenite and, further, in the presence of potassium dithio oxalate (KSOCCOSK).

14. In a process of flotation for the separation of metalliferous sulphides, the step of agitating and aerating an aqueous pulp containing said metalliferous sulphides, in the presence of a frothing and a collecting agent for one of the

sulphides, and further, in the presence of thioglycollic acids ( $\text{HSCH}_2\text{COOH}$ ) as a depressant.

15. In a process of flotation for the separation of metalliferous sulphides, the step of agitating and aerating an aqueous pulp containing said metalliferous sulphides, in the presence of a frothing and a collecting agent for one of the sulphides and, further, in the presence of alpha mercapto butyric acid ( $\text{HSC}_3\text{H}_6\text{COOH}$ ) as a depressant.

16. In a process of flotation for the separation of molybdenite from copper, iron, and similar sulphide minerals, the step of agitating and aerating an aqueous pulp containing the same, in the presence of a frothing and a collecting agent for the molybdenite and, further, in the presence of thioglycollic acid ( $\text{HSCH}_2\text{COOH}$ ) as a depressant.

17. In a process of flotation for the separation of molybdenite from copper, iron, and similar sulphide minerals, the step of agitating and aerating an aqueous pulp containing the same, in the presence of a frothing and a collecting agent for the molybdenite and, further, in the presence of alpha mercapto butyric acid ( $\text{HSC}_3\text{H}_6\text{COOH}$ ) as a depressant.

18. In a process of flotation for the separation of metalliferous sulphides, the steps of, first, subjecting an aqueous pulp containing the said metalliferous sulphides to inorganic acid conditioning, second, subjecting the acid conditioned pulp to lime conditioning sufficient to bring the pulp to an alkaline state, and, third, subjecting the so conditioned pulp to agitation and aeration in the presence of a frothing and a collecting agent for one of the sulphides and, further, in the presence of thioglycollic acid ( $\text{HSCH}_2\text{COOH}$ ) as a depressant.

19. In a process of flotation for the separation of metalliferous sulphides, the steps of, first, subjecting an aqueous pulp containing the said metalliferous sulphides to inorganic acid conditioning, second, subjecting the acid conditioned pulp to lime conditioning sufficient to bring the pulp to an alkaline state, and, third, subjecting the so conditioned pulp to agitation and aeration in the presence of a frothing and a collecting agent for one of the sulphides and, further, in the presence of alpha mercapto butyric acid ( $\text{HSC}_3\text{H}_6\text{COOH}$ ) as a depressant.

20. In a process of flotation for the separation of molybdenite from copper, iron, and similar sulphide minerals, the steps of, first, subjecting an aqueous pulp containing the said metalliferous sulphides to inorganic acid conditioning, second, subjecting the acid conditioned pulp to lime con-

ditioning sufficient to bring the pulp to an alkaline state, and, third, subjecting the so conditioned pulp to agitation and aeration in the presence of a frothing and a collecting agent for the molybdenite and, further, in the presence of thioglycollic acid ( $\text{HSCH}_2\text{COOH}$ ) as a depressant.

21. In a process of flotation for the separation of molybdenite from copper, iron, and similar sulphide minerals, the steps of, first, subjecting an aqueous pulp containing the said metalliferous sulphides to inorganic acid conditioning, second, subjecting the acid conditioned pulp to lime conditioning sufficient to bring the pulp to an alkaline state, and, third, subjecting the so conditioned pulp to agitation and aeration in the presence of a frothing and a collecting agent for the molybdenite and, further, in the presence of alpha mercapto butyric acid ( $\text{HSC}_3\text{H}_6\text{COOH}$ ) as a depressant.

22. In a process of flotation for the separation of metalliferous sulphides, the steps of, first, subjecting an aqueous pulp containing the said metalliferous sulphides to concentrated sulphuric acid conditioning, second, subjecting the acid conditioned pulp to lime conditioning sufficient to bring the pulp to an alkaline state, and, third, subjecting the so conditioned pulp to agitation and aeration in the presence of a frothing and a collecting agent for one of the sulphides and, further, in the presence of thioglycollic acid ( $\text{HSCH}_2\text{COOH}$ ) as a depressant.

23. In a process of flotation for the separation of molybdenite from copper, iron, and similar sulphide minerals, the steps of, first, subjecting an aqueous pulp containing the said metalliferous sulphides to concentrated sulphuric acid conditioning, second, subjecting the acid conditioned pulp to lime conditioning sufficient to bring the pulp to an alkaline state, and, third, subjecting the so conditioned pulp to agitation and aeration in the presence of a frothing and a collecting agent for the molybdenite and, further, in the presence of thioglycollic acid ( $\text{HSCH}_2\text{COOH}$ ) as a depressant.

HAROLD L. GIBBS.

#### REFERENCES CITED

The following references are of record in the file of this patent:

| UNITED STATES PATENTS |       |               |
|-----------------------|-------|---------------|
| Number                | Name  | Date          |
| 2,070,076             | Brown | Feb. 9, 1937  |
| 2,095,967             | Brown | Oct. 19, 1937 |
| 2,187,930             | Brown | Jan. 23, 1940 |